

March 12, 1940.

F. C. ELDER

2,192,901

METAL ARTICLE AND METHOD OF PRODUCTION

Filed Feb. 18, 1939



*Inventor*  
Flint C. Elder  
*By* John S. Jackson  
*Atty.*

## UNITED STATES PATENT OFFICE

2,192,901

METAL ARTICLE AND METHOD OF  
PRODUCTION

Flint C. Elder, Cleveland Heights, Ohio

Application February 18, 1939, Serial No. 257,203

2 Claims. (Cl. 174—132)

This invention relates to wires and the like, either individually or stranded, particularly to coated wires or strands that are adapted for use as electrical transmission lines, guy or stay wires, messenger wires, etc. The term "wire", as used herein, is intended to embrace all elongated metal bodies, of whatever cross-sectional shape, that are relatively flexible.

Wires to be used as overhead transmission lines are required to possess certain physical properties of electrical conductivity, tensile strength, and resistance to corrosion, in order to comply with commercial specifications. Commercial specifications provide for several different grades of wires or strands of this type in recognition of the fact that certain physical properties required for certain uses differ from those required for other uses, and that no single wire capable of providing the optimum as to one class of physical properties is capable of manifesting the optimum of physical properties of another class.

More specifically, it is recognized that the factors entering into the manufacture of a wire, best adapted from the standpoint of electrical conductivity, are not those which are conducive for the imparting of the best tensile characteristics, and vice-versa. For this reason, different commercial grades have been established to specify electrical conductors of the type required. The most common of these are three: E. B. B., B. B., and Steel. Where the electrical properties are non-essential or are secondary to high strength characteristics, a separate classification based on tensile properties is recognized, four in number: Common, Siemens-Martin, High-Strength, and Extra High Strength. In all of these grades the higher the tensile strength the poorer are the electrical properties, and vice-versa; the E. B. B. grade representing wires of the best electrical properties and of the lowest mechanical strength, and the Extra High Strength grade representing wires having the poorest electrical properties and the greatest mechanical strength.

It has, heretofore, not been considered possible to combine the best features of these several grades of wires in one, unitary conductor, since, as has been mentioned above, the factors entering into the manufacture of each, which will be discussed in full hereinafter, are such as to detract from certain of the physical properties, while enhancing some of the others.

Another very important factor, in considering wires of the type in question, is that of resistance to corrosion, which is usually provided for by the

addition of a protective coating, such as zinc, upon the surface of the wire. The coating, in addition to being initially impervious to corrosive influences, must be capable of remaining impervious; as, by being resistant to cracking when the wire is bent and flexed; and of a certain weight, prescribed by commercial standards, which will insure that the wire will be protected against corrosion for a predetermined period of time. Many of the physical properties entering into the acquisition of a good impervious coating, which will withstand flexing and other conditions of service without failing, are directly related to the physical properties contributing to the strength and electrical properties of the conductor, per se, and it is well established that those properties conducive to the acquisition of the best coating are not always provident of the best electrical and mechanical characteristics.

It is an object of the present invention to provide a wire of the class described which has electrical characteristics closely resembling those of the E. B. B. grade of conductors, while, at the same time, manifesting tensile strength characteristics comparable to those of the High Strength grade of wires.

It is another object to provide such a conductor with a corrosion resistant coating that is adherent, and, in weight and physical characteristics, that is as satisfactory from the commercial specification standpoint as the coatings to be found on any of the conductors or wires of the grades aforementioned.

It is still another object to provide a high tensile strength wire, low in carbon and other elemental inclusions, or, if relatively high in any of the latter, then, of greater tensile strength for the amount included than other wires of corresponding analysis, which has a hot-dipped coating of corrosion resisting metal firmly bonded thereto, and of an amplitude equal to or greater than coatings on corresponding wires of the same commercial class.

It is a further object to provide a wire of the class described whose tensile properties, electrical conductivity, and corrosion resistant coating will be of an higher order relative to the carbon, manganese, and other elemental inclusions, than any other wire of similar analysis of the corresponding commercial class.

Other objects and advantages will become apparent hereinafter after consideration is given to the specification wherein certain preferred embodiments of my invention are set forth.

The present invention constitutes a partial con-

tinuation of subject matter disclosed and claimed in my copending applications Serial Nos. 74,358 and 74,359, filed April 14, 1936, and Serial No. 79,207, filed May 11, 1936.

- 5 It is well known that the physical properties of steel, and particularly the tensile properties thereof, are developed by the inclusion of certain elements therein in relatively high amounts; for instance, carbon and/or manganese, present 10 in such amounts as to characterize the steel as a high carbon or high metalloid steel impart relatively high tensile values thereto. The manganese inclusions, ineffectual in and of themselves without the presence of carbon, serve to 15 enhance or augment the functions of the latter in raising the tensile properties of the steel; particularly, when a quench is employed after the carbon-manganese steel has been subjected to heat-treatment.
- 20 Another way to develop the tensile properties of steel, either complementary or supplementary to the chemical inclusions therein, is by working the metal at certain temperatures, and, particularly, by the so-called cold-working.
- 25 It is also well known that the inclusion of such elements as carbon and manganese, for the development of the tensile properties of steel, is accompanied by an increase in resistance to the 30 passage of electrical current through the steel in a fairly direct proportion to the amounts added. Furthermore, the quench sometimes employed to develop the ultimate in tensile properties of such steels is known further to impair the electrical properties thereof. It is for these 35 reasons that high strength steels are usually relatively poor conductors of electricity, and the low strength steels are the best conductors thereof.
- It has also hitherto been known that the presence 40 of certain elements, such as carbon, silicon, etc., in the metal to be coated, is conducive to the acquisition of a good hot-dipped coating of zinc, but here, again, the presence of such elements in any amount to be effective from a coating standpoint, is harmful to the electrical properties in that the elements increase the inherent 45 resistance of the steel to the passage of electrical current. On the other hand, cold-working is known to benefit the coating by augmenting its bond with the base metal, and by improving the 50 physical characteristics of the coating, so that it is better able to withstand flexing, and other strains and stresses encountered in service, without failing. Thus, a coating on low metalloid stock, which might otherwise be unsatisfactory, 55 is rendered satisfactory by substantial cold-reduction.
- I have discovered that a steel low in metalloids, which is the best from the standpoint of electrical properties, may be endowed with great 60 tensile strength by cold-working after it has been subjected to all treatment wherein it encounters heat in any substantial amount; as, for instance, in hot-galvanizing baths, annealing operations, etc. Such a steel, to meet the corrosion resistance requirements of the trade, must 65 be galvanized, which presupposes that the metal, if hot-galvanized, is subjected to the coating operation before cold-working to final size; or, else, that the coating operation is one that does not 70 involve the application of substantial temperature to the base metal; as, for instance, by electro-deposition. The present invention is principally concerned with the application of the corrosion resisting coating to the base metal by the 75 hot-dip method, which, in accordance with the

teachings of the invention, must be accomplished before the reduction to final size is undertaken. Cold-working a metal body after it has been coated, as by drawing hot-galvanized wire, effects a reduction in the thickness of the coating 5 at any given point on the surface of the metal, so that, if the end product is to have a sufficient thickness of coating to meet the commercial requirements, an extremely heavy coating must be initially provided before the drawing operation 10 is commenced.

Until the advent of the issuance of my U. S. Letters Patent No. 2,049,834, pertaining to methods of coating, there was no way known to the trade of applying a sufficiently heavy coating by 15 the hot-dip method, which coating could be subjected to the substantial reductions required to raise the tensile strength of the base metal, and still remain of sufficient amplitude per unit area of coated surface, after the drafting operation, 20 to meet the commercial standards and trade specifications. Electro-deposition methods presented the only possible alternative by which this could be done, but, by virtue of the relatively slow and expensive nature of this process, it is 25 rendered wholly impracticable from a commercial standpoint, and, so far as is known, has never been undertaken by anyone.

The single figure of the drawing is a side elevation with part shown in section of an apparatus 30 suitable for practicing the improved method and making the improved product.

Referring briefly to the apparatus, 6 represents a zinc pan such as shown in my above identified Letters Patent, and which is provided 35 with a burner 7 at an entrance end which maintains the zinc bath molten. The material A to be coated enters the molten zinc or galvanizing bath as described in my former patent and passes over guide sheaves 5, 8, 9, 10 and 12, as shown, 40 thence out over guide sheave 14 and through a die 16 which is effective to cold work the heavy galvanized coating accumulated on the wire in its passage through the bath. Thus the coated wire is cold worked after coating. The wire is 45 pulled through the apparatus by a suitable pulling block or take-up reel 15.

One preferred manner of carrying out my invention is by providing a steel rod or wire of low metalloid content; that is, low in carbon, 50 manganese, and other elements which are usually employed to improve physical properties (other than electrical) and coating characteristics of ferrous articles, which rod or wire is in size materially larger than that which is ultimately required, and upon which a heavy coating of metal is deposited, preferably by the hot-dip method; one suitable mode for effecting the latter being disclosed and described in my prior 55 patent, referred to above.

The over-size rod or wire coated in this manner is then subjected to cold-working, as by being drawn through reducing dies, until the required size is attained. Providing the reduction is substantial, as when something in excess of 60% reduction in cross-sectional area is had, the tensile properties of the material will be found to have been materially raised anywhere from 2 to 5 times their original values depending upon the extent of the reduction and the 65 composition of the material. The drafting practice will have been responsible for the establishment of a firm bond between the coating metal and the base metal as well as for the material improvement of the physical properties of the 70 75

coating metal. By virtue of the heavy coating initially put on, the wire after drafting will still retain a sufficiently heavy coating to meet the commercial specifications.

As a specific example of the present invention, a  $\frac{3}{8}$  inch diameter rod of the following analysis: carbon .05%, manganese .10%, phosphorus .005%, sulphur .023%, silicon .005%, and the balance substantially pure iron, was reduced to .192 inch diameter, representing a 74% reduction. This wire was then galvanized in hot zinc without annealing (other than that attendant upon being immersed in the molten zinc). A coating in the order of five ounces per square foot of zinc was applied representing a thickness of coating metal in the order of .015", thus increasing the over-all size of the wire from .192" to .207". The wire thus coated was then drawn to .072" over-all diameter, representing a total reduction of about 88%. This wire had a tensile strength of 135,000 pounds per square inch; an A. C. resistance of 5090 mile-ohm-pounds, yielding a skin effect A. C.-D. C. ratio of 1.165. Such values, as compared with the tensile strength of this magnitude, have heretofore not been obtained in wires of any known kind.

The following table shows how a wire prepared in accordance with the present invention (No. 12) compares with other wires of the same finished size made in accordance with standard commercial practices now in vogue.

of coating, expressed in ounces a square foot, as prescribed by the American Society for Testing Materials, are given below, with respect to the size of the wire, expressed in fractions of an inch diameter:

*ASTM specifications (A122-23) for galvanized wire strand*

| Size of wire inches diameter | Weight of coating (extra galvanized) ounces/square ft. surface | 10 |
|------------------------------|----------------------------------------------------------------|----|
| .207                         | .90                                                            |    |
| .188                         | .90                                                            |    |
| .165                         | .80                                                            |    |
| .145                         | .80                                                            | 15 |
| .120                         | .80                                                            |    |
| .104                         | .80                                                            |    |
| .093                         | .70                                                            |    |
| .080                         | .60                                                            |    |
| .072                         | .50                                                            |    |
| .062                         | .50                                                            |    |
| .052                         | .40                                                            | 20 |
| .041                         | .40                                                            |    |

Coatings lighter than these are not acceptable, for the sizes given, insofar as standard extra or double galvanized coatings are concerned. From this, it may be computed what the initial amount of coating must be to permit cold reduction to finished size after coating, still to maintain the requisite weight of coating metal. The extent of reduction permitted for any given weight of coating is determined by the application of the follow-

| 35 | Type of steel            |          |           | Treatment | Finish size diam.-inch                  | Lbs. per mile                     | Tensile strength | A. C. resistance |                     | D. C. resistivity |                        | Skin effect A. C.-D. C. ratio | 35         |        |       |
|----|--------------------------|----------|-----------|-----------|-----------------------------------------|-----------------------------------|------------------|------------------|---------------------|-------------------|------------------------|-------------------------------|------------|--------|-------|
|    | Grade                    | Carbon   | Manganese |           |                                         |                                   |                  | Mile ohm, lbs.   | Ohms per 1,000 feet | Mile ohm, lbs.    | Ohms per mile @ 68° F. |                               |            |        |       |
| 40 |                          |          |           |           |                                         |                                   |                  |                  |                     |                   |                        |                               | 40         |        |       |
| 45 | 1... BB.....             | .15 max. | Per cent  | Per cent  |                                         |                                   |                  | .109             | 167.3               | 57,500            | 8,807                  | 9.97                          | 5,609      | 33.528 | 1.570 |
|    | 2.....                   | .425     |           |           |                                         |                                   |                  | .109             | 167.3               | 95,000            | 8,860                  | 10.03                         | 7,535      | 45.038 | 1.175 |
|    | 3.....                   | .612     |           |           |                                         |                                   |                  | .109             | 167.3               | 199,000           | 9,408                  | 10.65                         | 8,833      | 52.80  | 1.065 |
|    | 4.....                   | .410     | .210      | .010      | Hot galvanized after annealing.         | .109                              | 167.3            | 74,000           |                     |                   |                        | 5,360                         |            |        | 45    |
|    | 5.....                   | .410     | .210      | .010      | Heat treated-drawn-then hot galvanized. | .109                              | 167.3            | 135,000          |                     |                   | 5,460                  |                               |            |        |       |
|    | 6.....                   | .350     | .20       | .10       | Hot galvanized after annealing.         | .109                              | 167.3            | 72,500           |                     |                   | 6,000                  |                               |            |        |       |
|    | 50                       | 7.....   | .350      | .20       | .10                                     | Hot galvanized without annealing. | .109             | 167.3            | 120,000             |                   |                        | 6,070                         |            |        | 50    |
|    | 8.....                   | .410     | .210      |           |                                         | .109                              | 167.3            | 125,000          | 7,800               | 8.83              | 5,610                  |                               |            |        |       |
|    | 9..... Steel.....        | .08-.10  | 25-.60    |           |                                         | .109                              | 167.3            | 59,000           | 9,630               | 11.0              | 6,500                  | 39                            |            | 1.48   |       |
|    | 10..... BB.....          | .08-.10  | 25-.60    |           |                                         | .1065                             | 160              | 59,000           | 8,760               | 10.4              | 5,580                  | 35                            |            | 1.57   |       |
|    | 11..... EBB.....         | .05 max. | .20       |           |                                         | .110                              | 167.4            | 49,500           | 8,720               | 9.88              | 4,980                  | 30                            |            | 1.75   |       |
| 55 | 12... Present invention. | .03-.04  | 12-.15    |           | Galvanized hard and drawn after.        | .109                              | 167.3            | 138,000          | 7,250               | 8.21              | 4,767-4,899            | 29.3                          | A.V.=4,833 | 1.48   | 55    |

From the foregoing table, it will be seen that I have provided a wire having tensile characteristic comparable to those of a high strength grade of wire, but which has electrical properties better than those specified for the E. B. B. grade of wire. In addition, the coating corresponds in thickness to that which is commercially known as an extra or double galvanized coating, for the finished size of wire in question (.109), which in weight, is .8 or more ounce per square foot of wire surface. Such a coating possesses the requisite physical values to permit its being flexed and bent without cracking, and is especially well bonded to the base metal, by virtue of the drafting to which it has been subjected.

For the class of wires in question, i. e., electric transmission lines and high strength guy or stay wires, the commercial standards for the weights

ing table, which represents data of empirical approximations, relative to the diminution of coating, expressed in ounces a square foot per percentage of reduction in cross-sectional area:

| Per cent-reduction cross-sectional area | Weight of coating in ounce/square foot | 65 |
|-----------------------------------------|----------------------------------------|----|
| Initial coating.....                    | 1.00                                   |    |
| 10.....                                 | 0.95                                   |    |
| 20.....                                 | 0.895                                  |    |
| 30.....                                 | 0.837                                  |    |
| 40.....                                 | 0.775                                  |    |
| 50.....                                 | 0.707                                  |    |
| 75.....                                 | 0.500                                  | 70 |

Since the conventional hot-dipped coating can not exceed 1.25 ounces a square foot of coated surface, it is easily computed from the foregoing

tables that the extent of reduction admissible on any coated wire of a given size is limited to fifty-nine percent (59%), if a weight of coating, definable as an extra-galvanized grade, is to be retained. Ordinary low metalloid steel, such as the present application is principally concerned with, has its tensile strength increased less than 35,000 pounds per square inch (32,450) by a fifty-nine percent (59%) reduction, which would be less than double its original tensile value. Ordinary high metalloid steel, (C=0.80%), would not be increased in tensile strength more than 60,000 pounds per square inch by such a reduction, representing an increase of less than double its original tensile value.

As the comparative table, listed above, shows, the steels similar to example No. 12 have tensile values appreciably more than double the original values of steels having carbon and manganese contents within the ranges given, since such steels usually start with a tensile value around 40,000 pounds per square inch as a maximum. Carbon steels, on the other hand, in which the carbon content approximates 0.80%, start with a tensile value of about 100,000 pounds per square inch. The low metalloid stocks will increase in tensile strength at the rate of about 550 pounds per square inch for every one percent (1%) reduction in cross-sectional area, while the carbon steel, suggested above, will increase about 1,000 pounds per square inch for every one percent (1%) reduction.

Thus, it will be seen 59 percent reduction is not sufficient to elevate the tensile strengths of these steels up to the desired values. Unless a heavier initial coating is provided, the tensile values must be limited to those procurable by such reduction. In accordance with the present invention, by starting with a heavy coating, such as was not possible of achievement by any hot-dip methods known to the trade prior to the issuance of my patent, above identified, I may carry the draughting practice to any point of reduction short of

100%, and finish with the weight of coating specified as standard for such finishing size, while enjoying an elevation of tensile strength that is not dependent upon elemental inclusions in the steel that adversely effect its electrical properties, nor dependent upon such processing, as quenching after heat treatment, from which impairment of the electrical properties likewise results.

While I have described one specific embodiment of my invention, it will be understood that I do not wish to be limited exactly thereto, since various modifications may be made without departing from the scope of my invention as defined by the following claims.

I claim:

1. A ferrous metal wire having a carbon content of .25 percent or less and a manganese content equal to or less than the carbon content, a heavy galvanized coating alloyed thereto, said coated wire cold worked subsequent to coating to produce a wire whose physical properties have a ratio of tensile strength, as expressed in pounds per square inch to its electrical resistivity, as expressed in pounds per mile ohm, higher than 25 to 1 with the actual direct current resistivity under 5,000 pounds per mile ohm and with the finished coating of an amplitude corresponding to that which is known as extra or double galvanized coating.

2. A ferrous metal wire having a carbon content of .25 percent or less and a manganese content equal to or less than the carbon content, a heavy galvanized coating alloyed thereto, said coated wire cold worked at least 59% subsequent to coating to produce a wire whose physical properties have a tensile strength of at least 125,000 pounds per square inch and with an actual direct current resistivity under 5,000 pounds per mile ohm and the finished coating being of an amplitude corresponding to that which is known as extra or double galvanized.

FLINT C. ELDER.